

May 24, 1938.

L. L. McGRADY ET AL

2,118,262

NONFOGGING CONTAINER FOR MOISTURE CONTAINING MATERIALS

Filed Oct. 4, 1934

Fig. 1.



Fig. 2.



Fig. 3



Fig. 4.



Inventors  
Leon L. McGrady & Charles G. Ritterhouse,

Newton M. Penning

By Daniel J. Mayne  
Attorneys

## UNITED STATES PATENT OFFICE

2,118,262

NONFOGGING CONTAINER FOR MOISTURE  
CONTAINING MATERIALS

Leon L. McGrady, Rochester, N. Y., and Charles G. Rittenhouse, Chicago, Ill., assignors, by mesne assignments, to Eastman Kodak Company, Jersey City, N. J., a corporation of New Jersey

Application October 4, 1934, Serial No. 746,852

4 Claims. (Cl. 206—44)

This invention relates to the art of packaging, and, more particularly to a non-fogging type of carton for the packaging of moisture-containing materials, such as fruit, berries, and other food products, as well as numerous other articles of commerce.

As is well known, there is a growing tendency among producers, especially producers of food-stuffs, fruits, vegetables and the like, to sell their products in package form rather than in bulk. This tendency has been the outgrowth, not only of a demand on the part of the public for more sanitary and attractive products, but also of recognition by the producers of the fact that packaged goods, generally speaking, keep better than when exposed in bulk. Regenerated cellulose and cellulose derivative thin sheeting has come greatly into vogue in the packaging art as a result of this modern trend and, so far as preservation of the products themselves are concerned, has been highly successful. However, all of the materials commonly used in packaging possess drawbacks which prevent them from being universally accepted. For example, it has been found that when moisture-containing materials, such as fruit, vegetables, berries and the like, are sealed up or enclosed in containers consisting of, or comprising, cellulosic material, such as regenerated cellulose or cellulose acetate, the moisture evolved from the packaged goods condenses and forms droplets on the inside surfaces of the container. In the case of regenerated cellulose the material absorbs the moisture and causes shrinkage or distortion which adversely affects the transparency of the material as well as producing an unsightly package.

On the other hand, cellulose acetate and similar types of cellulose derivative sheeting are much less subject to shrinkage and distortion, but due to the fact that this type of sheeting does not absorb moisture to any considerable extent, condensation of the moisture takes place within the package, thereby fogging or sweating the inside surfaces of cellulose derivative material by the deposition of minute droplets of water. This fogging action makes it impossible for the prospective purchaser to examine the contents of the package without opening it and thus seriously affects its salability. As is well known, it is the clear, glistening transparency of cellulose derivative and regenerated cellulose wrapping materials which give them their exceptional appeal to the public and it is obvious that anything which adversely affects this transparency, such as the condensation of moisture or the distortion of the

material, renders it unsatisfactory for use in a large number of fields in which it could otherwise be satisfactorily employed.

It is, accordingly, one of the objects of the present invention to provide a material which may be successfully employed in the manufacture of a non-fogging type of container for moisture-containing materials, especially such materials as fruit, vegetables, berries and the like. Another object is to provide a container for moisture-containing materials which is not susceptible to fogging or appreciable distortion from the effects of moisture. A further object is to provide a container, at least a portion of which consists of a cellulose derivative material, at least one side of which is provided with a coating which will prevent the accumulation of minute droplets of moisture in the form of fog. A still further object is to provide a substantially moistureproof container composed of, or including, a cellulose derivative material sheet material moistureproofed on one side and provided with an adherent coating of special character on the other side. A specific object of the invention is to provide a so-called window carton in which the window portion is composed of a cellulose derivative material, moistureproofed or unmoistureproofed, which is not subject to fogging or sweating due to the condensation of moisture within the package. Other objects will appear herein-after.

These objects are accomplished by the following invention which, in its broadest aspects, includes the provision of a cellulose derivative sheet material which has applied to one side thereof a coating comprising an adherent substance possessing a high degree of wettability and use of this material in the production of containers, either constituting the complete structure of the container, or a portion thereof, as would be the case in the manufacture of the so-called window type of carton.

In the following examples and description, we have set forth several of the preferred embodiments of our invention, but it is to be understood that they are included merely for purposes of illustration and not as a limitation thereof.

In the accompanying drawing.

Fig. 1 is a cross-section, on a greatly exaggerated scale, through a sheet of cellulose derivative material having on one side a highly wettable coating.

Fig. 2 is also an exaggerated cross-section through a sheet of material similar to the material of Fig. 1, but also including a moisture-

proof coating in addition to the wetable coating.

Fig. 3 is a perspective view of a window carton in accordance with our invention.

Fig. 4 is a perspective view illustrating a slightly 5 different embodiment of our invention.

As indicated above, we have discovered that the fogging or sweating of cellulose derivative containers made from, or including, cellulose derivative material may be prevented by coating 10 the inner surface of the material, that is the surface which is to be used on the inside of the container, with a thin film of material, preferably of an adherent nature, which possesses a high degree of wettability. Among the agents 15 which we have found to be especially valuable for this purpose are gelatin, agar agar, dextrin, egg albumen, casein and zein.

These materials are intended merely as illustrative, since many others of like character may 20 be employed. In fact any substance which is sufficiently adherent to adhere to cellulose derivative surfaces, which will form a thin transparent film thereon and which has a high degree of wettability is considered as coming within 25 the scope of our invention. It may be mentioned in this connection that wetable material may be applied directly to the surface of the cellulose ester sheeting or the sheeting may be provided with any of the customary substrata, such as 30 subs of cellulose nitrate or other cellulose esters.

According to one form of our invention, we may employ cellulose acetate sheeting as the material from which the container is to be made. This sheeting may be, either a thin material of 35 the order of .00088 to .015 inch in thickness, or a thicker type, such as a sheeting running from the .003 to .02 inch in thickness, depending upon the use to which it is to be put. If it is desired 40 merely to provide a window in a carton formed of waxed cardboard, for example, the sheeting may be of one of the thinner types. If, however, the whole container is to be composed of the material, it should preferably be of one of the thicker types of sheeting in order to withstand 45 the mechanical strains to which it is subjected in use. In some cases the cellulose derivative material may be cast in the form of a cylindrical or other type of container, provided with appropriate metallic or non-metallic end walls. 50 The last two types of containers are practically completely transparent.

Assuming that the sheet material is composed of cellulose acetate, it is coated in accordance 55 with our invention with one of the following compositions:

|                                           |                   |      |
|-------------------------------------------|-------------------|------|
| I. Gelatin                                | gms.              | 5    |
| Glacial acetic acid                       | c.c.              | 50   |
| Water                                     | c.c.              | 10   |
| 60 Methyl alcohol                         | c.c.              | 500  |
| Acetone                                   | c.c.              | 500  |
|                                           | Percent by weight |      |
| 65 II. Casein                             |                   | 1.0  |
| Ammonium hydroxide (28% aqueous solution) |                   | 2.0  |
| Sodium hydroxide                          |                   | 0.5  |
| Glycerine                                 |                   | 2.0  |
| Water                                     |                   | 24.5 |
| 70 Methyl alcohol                         |                   | 50.0 |
| Acetone                                   |                   | 20.0 |

The solution may be applied in any convenient manner known to those skilled in the art, such as 75 by subbing, beading, spraying, or the like. Re-

gardless of the particular method employed, there is deposited upon the surface of the cellulose derivative sheet a thin film or coating of adherent material of high wettability.

Referring to Fig. 1 of the drawing, A represents the base sheet of cellulose acetate, while B represents the coating of highly wetable material deposited thereon.

In Fig. 2 there is shown a slightly different form of the material in which the base sheet A is provided on one side with the wetable coating B and on the opposite side with a moistureproof coating C. The moistureproof layer may be composed of a mixture of gum and wax and applied to the sheeting in accordance with the procedure set forth in the copending application of N. F. Beach, Serial No. 551,491, filed July 17, 1931. The moistureproof coating may, however, comprise a layer of gum applied next to the sheeting, followed by a layer of wax in accordance with the procedure set forth in the U. S. patent to N. F. Beach and J. G. McNally No. 2,019,648. In some cases, the moistureproof coating may be applied to both surfaces of the sheeting, but in such cases the adherent, wetable layer is applied over the moistureproof coating in order that the moisture evolved from the moisture containing materials within the package may come in contact with the wetable layer.

In the manufacture of a carton in accordance 30 with our invention, one may first form the carton, as shown in Fig. 3, of waxed paper, cardboard, wood or similar material, P and provided with a cutout or window opening W. An appropriately sized "window" S is cemented around the edges 35 of the cutout portion W with an appropriate cement, thereby forming a substantially moisture-proof package.

In the form of our invention illustrated in Fig. 4, K represents a cellulose derivative container of 40 cylindrical form which may be fabricated from the cellulose derivative sheeting produced as described above, or may be cast from a suitable cellulose derivative molding composition and coated on the inside with a thin layer of the 45 adherent wetable material. The container K may be provided with appropriate metallic or non-metallic end closures E.

It is obvious that many changes in the specific 50 method of carrying out our invention are possible and we are, accordingly, not limited to any particular form thereof, except by the appended claims. Many types of cellulose derivative sheeting may be employed in making containers in 55 accordance with the invention. For example, we may employ moistureproofed or unmoisture-proofed cellulose acetate, cellulose propionate, cellulose butyrate, as well as certain of the mixed cellulose organic esters, such as cellulose acetate propionate, cellulose acetate butyrate, cellulose acetate stearate, and others. We may even use cellulose nitrate sheeting, although it is not to be preferred due to its high degree of inflammability and instability.

As stated above, our invention is particularly 65 characterized by the fact that containers or the window portions of window cartons made in accordance therewith will not fog or sweat due to the deposition of droplets of moisture. This feature of our invention is due to the highly wetable 70 character of the coating which we apply to the inner surface of the sheeting. An uncoated cellulose acetate sheet, for example, will condense the moisture within a package, in the form of minute droplets which appear to the eye as fog. This 75

cannot take place with the material described herein due to the fact that the moisture forms a continuous film over the surface of the wetable material, thus preserving substantially perfect 5 transparency of the original sheeting. This same effect of course takes place regardless of whether the cellulose derivative material is thick or thin, all that is necessary being that it shall be coated on its inner surface with the adhesive film of wetable material.

Our invention is also characterized by the fact 10 that the material described herein is not subject to wrinkling or unsightly distortion due to shrinkage or swelling, which is one of the most outstanding 15 defects of regenerated cellulose sheeting when used for packaging moisture-containing materials.

It will readily be seen that when we employ a 20 moistureproof type of sheeting, in accordance with the invention, we are enabled to maintain the moisture within the package at a constant 25 value, since the moisture cannot escape through the moistureproof sheeting. Notwithstanding that the moisture is retained within the package, as indicated above it does not give rise to fogging or unsightly distortion due to the presence of the wetable film thereon.

Our invention is of especial value in the packaging of fruits, vegetables, berries, and other food 30 products containing in their natural state a considerable amount of moisture. It is now possible by the use of packages produced as described herein to package almost any type of moisture-containing materials with highly satisfactory results. This opens up a large field which has, 35 heretofore, been closed to the manufacturer of transparent cartons, and, likewise, has solved for the producer of many types of grown and artificially manufactured food products the problem 40 of packing and shipping such products in transparent containers of the type which have been so widely successful in other fields.

Having thus described our invention, what we declare is new and desire to secure by Letters 45 Patent of the United States is:

1. A window-type carton adapted for packaging moisture containing materials without fogging of the window portion thereof, comprising side and end walls at least one of which has a window opening therein, a permanently transparent sheet of cellulose derivative material which is relatively non-absorptive of moisture closing the window opening, said sheet having on its inner surface a thin, adherent, non-fogging coating of solid, transparent, relatively moisture absorptive material.

2. A window-type carton adapted for packaging moisture containing materials without fogging of the window portion thereof, comprising side and end walls at least one of which has a window opening therein, a permanently transparent sheet of cellulose derivative material which is relatively non-absorptive of moisture closing the window opening, said sheet having on its inner surface a thin, adherent, non-fogging coating of 20 gelatin.

3. A permanently transparent, non-fogging container for moisture containing materials comprising a hollow cylindrical member provided at its ends with caps, such hollow member consisting of a permanently transparent sheet of cellulose derivative material which is relatively non-absorptive of moisture having on its inner surface a thin, adherent, non-fogging coating of solid, transparent, relatively moisture absorptive material.

4. A window-type carton adapted for packaging moisture containing materials without fogging of the window portion thereof, comprising side and end walls at least one of which has a window opening therein, a permanently transparent sheet of cellulose derivative material which is relatively non-absorptive of moisture closing the window opening, said sheet having on its inner surface a thin, adherent, non-fogging coating of 35 solid, transparent, relatively moisture absorptive material and having on its outer surface a moisture-proof coating.

LEON L. McGRADY.

CHARLES G. RITTENHOUSE.

45